

## UNITED STATES PATENT OFFICE.

LEON W. EBERLIN, OF ROCHESTER, NEW YORK, ASSIGNOR TO EASTMAN KODAK COMPANY, OF ROCHESTER, NEW YORK, A CORPORATION OF NEW YORK.

## PROCESS OF REMOVING PYRIDINE FROM NITROCELLULOSIC MATERIALS.

No Drawing.

Application filed February 11, 1925. Serial No. 8,575.

To all whom it may concern:

Be it known that I, LEON W. EBERLIN, a citizen of the United States of America, residing at Rochester, in the county of Monroe and State of New York, have invented certain new and useful Improvements in Processes of Removing Pyridine from Nitrocellulosic Materials, of which the following is a full, clear, and exact specification.

10 This invention relates to processes of removing pyridine from cellulosic materials which are impregnated therewith. One object of the invention is to provide a process for removing pyridine from these materials, 15 such as solid colloidized nitrocellulose, for example, in a rapid, thorough and relatively inexpensive manner. Other objects will hereinafter appear.

In reducing the viscosity characteristics of 20 nitrocellulose, especially solid colloidized nitrocellulose, such as pyroxylin waste and film scrap, it has been proposed to use solutions of pyridine which thoroughly impregnate the material. Even though the latter is 25 in a solid condition it is sufficiently softened so that the pyridine enters the interior thereof. Pyridine has an odor which is objectionable to many people, and even small traces of it give off a detectable smell. 30 Moreover, any considerable amounts of it in nitrocellulose tend to bring about a molecular transformation which may proceed too far. It is, therefore, highly desirable to provide a rapid, simple and inexpensive 35 process for eliminating this material from the treated nitrocellulose. While I have referred particularly to the removal of pyridine from solid colloidized nitrocellulose, the method is equally applicable to any material, 40 especially cellulosic material, of an analogous nature.

I have found that pyridine may be successfully removed by subjecting the material containing it to a chlorinating agent. I prefer to have present also a penetrant, which 45 facilitates the action between the chlorine and the pyridine. While various chlorinating agents may be employed, I find that the simplest one is chlorine gas itself. As a 50 penetrant I may employ a solvent properly toned by a diluent so that it does not dissolve the material but merely softens the latter to permit the action to take place. In the case of nitrocellulose a 20% aqueous solution of a usual solvent, such as acetone or

methyl alcohol or methyl acetate, is useful. But the proportion can be varied through a considerable range, provided the nitrocellulosic material is not dissolved or rendered so gummy as to stick together into an unmanageable mass. 60

While the action may be facilitated or speeded up by the use of heat, this is unnecessary, as useful rapidity is obtained at room temperature. The process is, of course, conducted in a vessel which is practically proof against the action of chlorine. 65

While I shall now describe one form of my invention by way of example, it will be understood that the invention is not restricted to the details of this illustration except as indicated in the appended claims. Nitrocellulosic material, especially one containing solid colloidized nitrocellulose, associated or not with high-boiling compounds like camphor and butyl alcohol, such as pyroxylin waste or film scrap, which has been impregnated with pyridine in previous operations, is immersed in a bath comprising a 20% aqueous solution of acetone. After the penetrant, acetone, 70 has been allowed to act on the material to slightly swell the latter, chlorine gas is bubbled up through the liquid in intimate contact with the material until there is a distinct odor of chlorine when the gas supply is 75 shut off.

The film is then left in the chlorinated bath until a test shows that the pyridine has been sufficiently decomposed into harmless and readily removable substances. The time 80 of this treatment is, of course, variable and depends upon the concentration of pyridine in the material, the extent to which the material has been comminuted before the treatment, and upon the strength of the penetrant, as well as the temperature. Working at room temperature with comminuted film scrap the action is sufficiently complete in about 30 minutes. 85

When the action is finished, the chlorinating bath is drained from the material and the latter washed in several changes of water. It is then treated, say by immersion, in an anti-chlor solution. The simplest and most inexpensive bath of this nature is one of sodium thiosulfate, say a 5 to 10% aqueous solution.

This acts very quickly. Finally the material is washed to remove the thiosulfate. This can be done continuously in cold run-

ning water or by treatment in successive treatments of cold water. In the latter case the water may be warmed to hasten the action.

5 Having thus described my invention, what I claim as new and desire to secure by Letters Patent is:

1. The process of removing pyridine from cellulosic material which is impregnated 10 with the same, which comprises treating said material with a chlorinating agent to decompose the pyridine and then treating the material with an anti-chlor solution.

2. The process of removing pyridine from 15 cellulosic material impregnated with the same, which comprises treating said material with a chlorinating agent in the presence of a penetrant to decompose the pyridine and treating the material with an anti-chlor solution.

3. The process of removing pyridine from 20 solid colloidized nitrocellulose containing the same, which comprises treating the said nitrocellulose with a chlorinating agent in the presence of a mixture of water and a penetrant until the pyridine is substantially 25 decomposed, removing the nitrocellulose from the mixture and treating the same with an anti-chlor solution until any free chlorine is neutralized.

4. The process of removing pyridine from 30 solid colloidized nitrocellulose containing the same, which comprises treating the same with a chlorinating agent in the presence of 35 a penetrant until the pyridine is substantially decomposed, thereafter treating the nitrocellulose with an anti-chlor solution to remove any free chlorine and finally washing the nitrocellulose to remove the compounds formed by the previous steps.

40 5. The process of removing pyridine from solid colloidized nitrocellulose containing the same, which comprises immersing said nitrocellulose in an aqueous bath containing sufficient nitrocellulose solvent to act as a penetrant without dissolving said nitro-

cellulose, bringing chlorine gas into contact with said nitrocellulose while thus immersed, allowing the chlorine to decompose the pyridine, separating the nitrocellulose from 50 said bath, treating it with an anti-chlor solution to neutralize any free chlorine remaining therein, and finally washing the nitrocellulose to thoroughly remove the compounds formed in the previous steps.

6. The process of removing pyridine from nitrocellulose film scrap containing the same, which comprises immersing said scrap, while in small pieces, in a 20% aqueous solution of a nitrocellulose solvent, bubbling chlorine gas through said solution until there is a distinct odor of chlorine when the gas supply is shut off, allowing the chlorine bath to complete the decomposition of the pyridine in the scrap, draining the bath from the scrap, rinsing the same, and then immersing it in a bath of thiosulfate of an alkali metal until any remaining chlorine is neutralized, and finally washing the scrap to remove the compounds introduced 65 by the preceding steps.

7. The process of removing pyridine from nitrocellulose film scrap containing the same, which comprises immersing said scrap in a 20% aqueous solution of acetone and 70 permitting the scrap to swell slightly, bubbling chlorine gas through the bath into contact with the scrap, until a distinct odor of chlorine remains when the gas supply is shut off, allowing said chlorine in the 75 bath to complete the decomposition of the pyridine in the scrap, draining the bath from the scrap and washing the latter in water, immersing the scrap in a bath of sodium thiosulfate to neutralize any remaining chlorine, and finally washing the scrap with water until the compounds introduced by the previous steps are substantially removed.

Signed at Rochester, New York, this 5th day of February 1925.

LEON W. EBERLIN.